

Patented Apr. 27, 1926.

1,582,257

# UNITED STATES PATENT OFFICE.

DE RALPH FRIZELL, OF LOS ANGELES, AND BERT ALLEN STAGNER, OF BERKELEY, CALIFORNIA, ASSIGNORS TO UNION OIL COMPANY OF CALIFORNIA, OF LOS ANGELES, CALIFORNIA, A CORPORATION OF CALIFORNIA.

## PREPARING SOLUBLE OILS.

No Drawing.

Application filed April 1, 1922. Serial No. 548,847.

To all whom it may concern:

Be it known that we, DE RALPH FRIZELL and BERT ALLEN STAGNER, citizens of the United States, and residents, respectively, 5 of Los Angeles, in the county of Los Angeles and State of California, and of Berkeley, in the county of Alameda and State of California, have invented certain new and useful Improvements in Preparing Soluble 10 Oils, of which the following is a specification.

Our invention relates to making soluble oils or emulsifiers, such being oils or oil compounds capable of ready dispersion in cold 15 water with slight agitation, whereby a stable emulsion is formed.

One of the principal objects of our invention is the use of waste products from refining crude petroleum, the same being the 20 naphthenic acids or their soaps, of which the sodium naphthenates are especially preferred.

Naphthenic acids may be obtained from the waste alkali washes in petroleum refineries, being contained in the same as partly 25 saponified products, in a number of ways, such as are described in the copending applications of L. L. Rebber, Serial Number 559,612 filed May 9th, 1922, and De R. Fri- 30 zell, Serial Number 559,614 filed May 9th, 1922.

They are oxidation products of the naphthene series  $C_nH_{2n}$ , which are naturally present in petroleum distillates or are formed 35 by the oxidizing action of the sulphuric acid used in purifying petroleum products or by other oxidizing agents, and consist of a hydrocarbon radical, or a substituted hydrocarbon radical, in combination with a carboxyl group of which hexahydrobenzoic acid,  $C_6H_{11}COOH$ , may be taken as illustrative.

In the refining of petroleum distillates, the distillates are treated with sulphuric acid and the acid sludge, containing the sulphonic acids and sulphonates, are drawn off, naphthenic acids being formed at the same time and remain in the distillate. The distillate is then treated with an alkali, such 45 as the alkali metal hydroxides, preferably sodium hydroxide, and the alkali sludge containing the naphthenic acids and naphthenates is drawn off.

The naphthenic acids and naphthenates are present in the waste alkali in a partly 55 saponified condition, and in order to recover them therefrom, we preferably treat the waste alkali with sulphuric or other suitable acid, whereupon the naphthenates are broken up into naphthenic acids and together with 60 the naphthenic acids previously present are thrown out of solution and recovered in any suitable manner.

Saponification is effected by treating with 65 strong sodium hydroxide, added in small amounts to avoid excess, and the sodium naphthenic soaps so formed are then heated and stirred to drive off excess moisture and further mixed with cresol in the proportion of about one part cresol to four parts of the 70 sodium naphthenates by volume, but we do not hereby limit ourselves to the above proportions inasmuch as we have found other proportions to be equally valuable, the above mentioned proportions being merely illustrative.

The resulting product is mixed in varying proportions with mineral oils to form a soluble oil, the proportions varying with the mineral oil taken for a specific use and we 80 find we can use a light oil, such as kerosene, or a heavy oil such as a crude oil, with equally good results for any particular class of work.

The soluble oils thus produced, with slight 85 agitation are readily emulsified in water, forming stable emulsions, being miscible therein in any proportion.

The emulsions are used in the treatment of wools, sprays for fruit trees, sheep dips, 90 cordage oils, a substitute for Turkey-red oils, lubricants, etc.

Corresponding results are obtained by the compounding of sodium naphthenates with cresol and an oil of vegetable or animal 95 origin, such as cottonseed or fish oils, but in general the stability of emulsions made from soluble oils of purely mineral origin is greater than that made from oils made from part mineral and part vegetable or animal origin, 100 and we preferably make our soluble oils with the sodium naphthenates obtained from a particular stock and a distillate prepared from that stock, or a similar stock.

However, in either case, the use of cresol 105 with naphthenates increases the stability of

emulsions, in comparison to their stability when prepared by other methods, and we may use cresol, the acids of cresol or their salts.

5 Cresol is generally obtained from coal or wood tar and has the formula  $\text{CH}_3\text{C}_6\text{H}_4\text{OH}$ , thus being an aromatic hydroxyl derivative which has valuable antiseptic properties which make our product especially valuable for the production of thread cutting emulsion. However, the function of cresol in our invention is that of a common solvent for the oil and the naphthenic soap whereby emulsions can be made with water 15 which are rendered relatively more permanently stable, its antiseptic qualities being purely incidental to its use in the process described.

Commercial cresol contains three isomeric 20 forms and according to one authority (Lunge, Coal Tar and Ammonia, Vol. II, pp. 772) has the following constitution:

|                                                       | Per cent. |
|-------------------------------------------------------|-----------|
| 25 Iso cresols                                        | 95        |
| Phenol                                                | 2         |
| Xylenes                                               | 1         |
| Higher phenols, pyridene bases, residues, water, etc. | 2         |

30 In view of this content of aromatic hydroxyl derivatives, the term "cresol" where used in the claims is intended to include all equivalents of cresol or contained derivatives.

35 The emulsions made from our soluble oils easily pass all Government tests, which require that polished brass or copper must not turn green after standing in an emulsion twenty-four hours, and that polished steel 40 must not be corroded after standing in an emulsion two weeks.

We claim:

1. The process of preparing soluble oils which consists in saponifying naphthenic acids, mixing the naphthenates with cresol and dissolving the resulting compound of naphthenates and cresol in an oil. 45

2. The process of preparing soluble oils which consists in saponifying naphthenic acids with a caustic alkali, mixing the alkali naphthenates with cresol and dissolving the resulting compound in an oil. 50

3. The process of preparing soluble oils which consists in saponifying naphthenic acids with sodium hydroxide, mixing the

sodium naphthenates with cresol and dissolving the resulting compound in an oil.

4. The process of preparing soluble oils which consists in saponifying naphthenic acids with sodium hydroxide, mixing the sodium naphthenates with cresol and dissolving the resulting compound in a mineral oil. 60

5. The process of preparing soluble oils which consists in saponifying naphthenic acids, with sodium hydroxide and adding about one part of cresol to about four parts by volume of the resulting naphthenic soaps then dissolving the resulting compound in a mineral oil. 65

6. The method of making an emulsion from hydrocarbon oils which consists in mixing sodium naphthenic soaps with cresol dissolving the mixture in the aforesaid oils and dispersing the resulting compound in water. 70

7. The method of making an emulsion from hydrocarbon oils, which consists in mixing sodium naphthenic soaps with cresol in the proportion of about one part of cresol 80 to about four parts by volume of sodium naphthenic soaps, dissolving the mixture in the hydrocarbon oil then dispersing the resulting compound in water.

8. A soluble oil comprising an alkali metal naphthenate, cresol and oil. 85

9. A soluble oil comprising sodium naphthenate, cresol and an oil.

10. A soluble oil comprising sodium naphthenate, cresol and a mineral oil. 90

11. A soluble oil comprising about one part of cresol to four parts by volume of sodium naphthenate, and a mineral oil.

12. An emulsion comprising sodium naphthenate, cresol, mineral oil and water. 95

13. An emulsion comprising cresol, sodium naphthenate, a mineral oil and water; the cresol being in the proportion of about one part of cresol to four parts of sodium naphthenate by volume. 100

Signed at Los Angeles, in the county of Los Angeles, and State of California, this 27th day of March 1922.

DE RALPH FRIZELL.

Signed at Oleum, in the county of Contra Costa, and State of California, this 25th day of March, 1922.

BERT ALLEN STAGNER.